

# United States Patent [19]

Kamigaito et al.

[11] 3,915,721

[45] Oct. 28, 1975

[54] RESISTOR FOR SPARK PLUG

[75] Inventors: **Osami Kamigaito; Hideyuki Masaki; Masami Oki**, all of Nagoya; **Masatoshi Suzuki, Kariya; Yasuo Nakamura**, Nagoya, all of Japan

[73] Assignees: **Nippondenso Co., Ltd.; Kabushiki Kaisha Toyota Chuo Kenkyusho**, both of Japan

[22] Filed: Sept. 20, 1973

[21] Appl. No.: 399,275

[30] Foreign Application Priority Data

Sept. 22, 1972 Japan..... 47-95439

[52] U.S. Cl. .... 106/46; 117/124 A; 252/518

[51] Int. Cl.<sup>2</sup> .... C04B 33/26

[58] Field of Search..... 106/46, 45, 39.5; 117/124 A; 252/518

[56] References Cited

UNITED STATES PATENTS

2,152,655 4/1939 McDougal et al. .... 106/46 X

|           |         |                     |           |
|-----------|---------|---------------------|-----------|
| 2,853,392 | 9/1958  | Bousky .....        | 106/46    |
| 2,864,773 | 12/1958 | Counts et al.....   | 252/503   |
| 2,885,521 | 5/1959  | Fotland .....       | 106/46 X  |
| 3,062,668 | 11/1962 | Pierrot et al.....  | 106/39.5  |
| 3,235,655 | 2/1966  | Counts et al.....   | 252/520 X |
| 3,658,583 | 4/1972  | Ogawa et al.....    | 106/46 X  |
| 3,660,124 | 5/1972  | Yoshioka et al..... | 106/46 X  |

## FOREIGN PATENTS OR APPLICATIONS

1,213,621 11/1970 United Kingdom..... 106/46

Primary Examiner—Allen B. Curtis

Assistant Examiner—Thomas A. Waltz

Attorney, Agent, or Firm—Cushman, Darby & Cushman

[57]

## ABSTRACT

There is provided a resistor for spark plugs used in an internal combustion engine. The resistor comprises a resistance material consisting of tantalum oxide, tin oxide and antimony oxide in proper proportion by weight.

5 Claims, 8 Drawing Figures

FIG. I



FIG.2



FIG. 3



FIG. 4





FIG. 6



FIG. 7



FIG. 8



## RESISTOR FOR SPARK PLUG

The present invention relates to spark plugs which do not cause communication radio wave interference, and more particularly the present invention relates to a resistor of 3 to 20 kiloohms used with internal combustion engine spark plugs of the type which are provided with a center electrode.

In the past, spark plugs heretofore used in internal combustion engines have been of the type which employ a low resistance center electrode. A disadvantage of this type of spark plugs is that the radio waves generated upon the production of a spark at the spark plug in service gives rise to communication radio wave interference. With the recent development of communications, the consideration of remedial measures against radio wave interference has become increasingly important. In the case of the spark plugs for internal combustion engines, the insertion of a resistor in the electric circuit for the spark plug has been proposed as a means of suppressing the interference and various methods have been used for this purpose. These methods may be divided into two classes: one in which the resistor is inserted in the spark plug itself and the other in which the resistor is inserted in the high tension cable for the ignition circuit.

In these remedial measures against radio wave interference, it is required that a resistor be used whose resistance values is in the range between 3 to 20 kiloohms at temperatures ranging from the normal temperature up to 400°C.

In the past, spark plugs of the type having a conducting seal composed of a conductive material bonded with a highly heat resisting glass material of low melting point have been extensively used.

Such a conducting glass seal is prepared by mixing a resistance material such as a powdered metal (e.g., copper, iron nickel or nickel-chromium type metal) or carbon or a powdered low resistance metal oxide (zinc oxide, barium borate, chrome dioxide, chrom trioxide, nickel oxide or the like) with a powdered low melting glass such as borosilicate type glass, heating the mixture up to a temperature higher than the softening temperature of the glass, and compressing and sealing it in place with the electrode, thus producing a resistor with this sealed glass member.

However, the specific resistances of spark plug resistors produced in this manner are all lower than 0.01 kΩ-cm and the insertion of such a low resistance resistor in the spark plug can provide only a resistance of lower than 0.1 kΩ which practically has no noise suppressing effect. While the amount of glass in this resistor may be increased to produce a high resistance resistor for spark plugs, the specific resistances of resistors that may be produced by slightly changing the amount of glass are subject to extremely wide variations ranging from 0.01 to 1000 kΩ-cm and thus their manufacture is impractical. Further, in the high resistance spark plug resistor produced by increasing the amount of glass, the resistance material disperses in the glass material and thus the resistor is structurally unstable and not well suited for practical use.

With a view to overcoming the foregoing difficulty, it is the object of the present invention to provide a resistor for spark plugs which is composed of a high resistance material having a novel composition and which

has a high resistance of 3 to 20 kiloohms that is effective in suppressing noise.

The resistor for spark plugs according to the present invention has among its great advantages the fact that the specific resistance of the resistor is readily controlled by adjusting the amount of added tantalum oxide and therefore the resistance value can be easily increased without resorting to any complicated procedure of increasing the amount of glass to obtain an increased resistance value. The range of variations of the resistance value of the resistor is narrow and it has a structural stability with the required resistance value of 3 to 20 kiloohms. Further, a wider range of sintering temperatures usable in the manufacture of this resistor is a great convenience to the manufacture thereof.

Other objects, advantages and features of this invention will become readily apparent from considering the following detailed description taken in conjunction with the accompanying drawings, in which:

20 FIGS. 1 to 6 are graphs for the experimental examples of this invention, in which:

FIG. 1 shows the relationship between the amount of antimony oxide in a resistor produced by combining tin oxide and antimony oxide together with a glass and the 25 change in resistance before and after spark discharge;

FIG. 2 shows the relationship between the amount of antimony oxide in a resistance material consisting of tin oxide and antimony oxide and the specific resistance thereof;

30 FIG. 3 shows the relationship between the spark discharge period and the specific resistance of a resistor according to the present invention;

FIG. 4 shows the relationship between the temperature and the specific resistance of the resistor of FIG. 3;

35 FIG. 5 shows the relationship between the amount of tantalum oxide in resistance materials and the specific resistance and the resistance value of resistors;

FIG. 6 shows the relationship between the amount of 40 glass in the resistor and the specific resistance thereof;

FIG. 7 is a sectional front view of a spark plug having sealed therein the resistor according to the present invention; and

45 FIG. 8 is a sectional front view of another spark plug in which the resistor of this invention is provided in place in the form of a rod-shaped resistor.

A novel spark plug resistor provided in accordance with the present invention is produced by sintering (bonding), with a low melting glass, a resistance material having the composition: tantalum oxide 1-30 % by weight, tin oxide 63-98 % by weight and antimony oxide 0.7-9.9 % by weight.

50 In accordance with the present invention, the tantalum oxide consists of tantalum pentoxide ( $Ta_2O_5$ ), tin oxide consists of tin monoxide ( $SnO$ ) or tin dioxide ( $SnO_2$ ), antimony oxide consists of antimony trioxide ( $Sb_2O_3$ ) or antimony tetroxide ( $Sb_2O_4$ ) and the low melting glass consists of borosilicate type glass. While the resistance material is composed of these oxide of tantalum, tin and antimony in the previously mentioned composition ranges, this composition is determined on the following reasons.

55 In other words, in order that this resistance material may ensure a stable performance of the spark plug, that is, the change of the resistance value of the resistor due to the repeated ignition may be reduced, it is essential that the resistance material contains tin oxide and anti-

mony oxide in proper proportions. Namely, the resistance material should comprise between 90-99 % (by weight and this is the same with all other percentages) of tin oxide and between 10-1% of the antimony oxide. If the antimony oxide content is less than 1%, the aforesaid stable performance of the spark plug is deteriorated. While the stable performance is ensured with the antimony oxide content higher than 1 % if this content is higher than 10 %, there is an inconvenience in that when the resistance material is sintered and bonded using the glass, bubbles produced enter into the glass phase. However, there is a problem that mere bonding of the two constituents with the glass results in a resistor whose specific resistance is as low as about  $10^{-5}$  -  $10^{-3}$  k $\Omega$ -cm and it is difficult to produce the desired resistor. The addition of tantalum oxide is therefore necessary to produce the desired resistance material. The proportion of tantalum oxide to be mixed is such that a total amount of tin oxide and antimony oxide is between 70-90 % and the remaining tantalum oxide content is between 30-1 %. If the tantalum oxide content is less than 1 %, in the case of an ordinarily employed spark plug of practical size, it is difficult to obtain a resistor of over 3 kilohms. On the other hand, if this content is higher than 30 %, it is difficult to obtain a resistor of less than 20 kilohms. As will be seen from this fact, the preferred proportions of the constituents in the composition of the resistance material as a whole are ultimately determined, as mentioned previously, as follows: tantalum oxide 1-30 %, tin oxide 63-98 %, antimony oxide 0.7-9.9 %.

Further, in the resistor according to the present invention, the proportions of the resistance material and the low melting glass should preferably be such that the resistance material is in the range 40-90 % and the glass is in the range 60-10 %. When the amount of glass exceeds 60 %, the glass enters between the particles of the resistance material thus increasing the resistance value considerably, while even a slight change in the amount of glass results in a large variation of the resistance value and it is difficult to obtain a resistor with the desired resistance (FIG. 6). The glass content should preferably be greater than 10 % in order to ensure the bonding of the resistance material. Further, if the resistor is sealed in the spark plug, the amount of the glass should preferably be in the range 20 % or above from the gastight point of view.

The resistor according to the present invention may be utilized by sealing it in the spark plug between its center electrode and central conductor as mentioned above, or alternately the resistor may be inserted in the spark plug in the form of a solid resistor or it may be placed in the high tension conductor cable for the ignition circuit outside of the spark plug.

When the resistor is to be sealed in the spark plug, as shown in FIG. 7, a resistor 2 is compressed and sealed between a center electrode 3 inserted in the lower end of the bore formed in an insulator 4 and a central conductor 1 inserted above the center electrode 3, thereby joining them together. In this case, therefore, the resistor serves not only to suppress communication radio wave interference, but also to provide the required electric conduction between the center electrode 3 and the central conductor 1 and hermetically seal them to the insulator. In FIG. 7, numeral 5 designates a housing, numeral 6 a ground electrode.

In the spark plug shown in FIG. 8, the resistor according to this invention is inserted in the form of a rod-shaped solid resistor. A center electrode 3' inserted in the lower end of the bore formed in an insulator 4' is enclosed by a conventional high-conductive substance 7 and a metal conductor 9 is fixedly placed above the substance 7. Disposed above the metal conductor 9 is a spring 8 and a resistor 2' according to this invention is placed between this spring 8 and a central conductor 1'. The central conductor 1' is screwed into the bore of the insulator 4' to securely hold the resistor 2' in place. As a result, the resistor 2' is not required to serve as a seal as in the spark plug shown in FIG. 7.

As described hereinbefore, the resistor according to the present invention comprises a resistance material composed of the above-mentioned three constituents, i.e., tantalum oxide, tin oxide and antimony oxide and bonded with a low melting glass. This resistor is produced according to the following procedure: tin oxide and antimony oxide are mixed and then heated to a high temperature to cause reaction between the two elements. The resultant reaction substance is added with tantalum oxide and reheated to an elevated temperature to cause reaction therebetween. A low melting point glass such as borosilicate glass is added to the ternary resistance material in fine powder form and a small quantity of an adhesive substance such as polyvinyl alcohol is also added. These elements are thoroughly mixed together to obtain a substantially uniform mixture. This mixture is then placed in the spark plug or alternately it is placed in a molding form, heated to an elevated temperature to soften the glass and then cooled to produce a resistor. When this resistor is to be placed in the spark plug, as in the case of a conventional sealed-resistor type spark plug, the abovementioned mixture is placed, as shown in FIG. 7, between the center electrode 3 and the central conductor 1 and a pressure is applied to the central conductor 1 to compress and seal the resistor in place at an elevated temperature, thereby producing the spark plug having the resistor 2 sealed between the central conductor 1 and the electrode 3. On the other hand, when the abovementioned mixture is to be placed in the molding form, the mixture is inserted for example in a cylindrical molding form, heated and then cooled to produce a cylindrical resistor. This resistor is inserted, as the resistor 2', between the conductor 9 electrically connected to the center electrode 3' and the central conductor 1' as shown in FIG. 8.

The effects of the various mixing proportions of the above-described resistance material and the glass will be described with reference to the following experimental examples. In the following experimental examples, the tin oxide, antimony oxide and tantalum oxide used consisted of  $\text{SnO}_2$ ,  $\text{Sb}_2\text{O}_3$  and  $\text{Ta}_2\text{O}_5$ , respectively, and the glass consisted of borosilicate glass. As will be described in greater detail in connection with the description of the experimental examples, each of the resistors in the experimental examples was produced by mixing given amounts of the resistance material and the glass together, heating the mixture to soften the glass and then bonding the resistance material with the glass.

#### Experimental EXAMPLE 1

The test results on the stability of the binary system resistance materials consisting of tin oxide and antimony oxide will be explained with reference to FIG. 1.

In other words, each of the resistance materials produced by mixing tin oxide and antimony oxide in various proportions was sintered using the low melting glass and the resultant rod-shaped resistor placed in the spark plug in the form of a solid resistor as shown in FIG. 8 was tested by the resistor load life testing method according to JIS 5102. FIG. 1 shows the results of the tests on the changes in the resistance values of the resistors before and after the discharging of spark for a period of 250 hours. In FIG. 1, the ordinate represents the rate of change (%) of the resistance value and the abscissa represents the amount of the added antimony oxide (%) in the binary resistance materials consisting of tin oxide and antimony oxide.

As will be seen from FIG. 1, if the antimony oxide content is less than 1 %, the change of the resistance value before and after the test is extremely great and the resultant resistor cannot be put in any practical use. On the other hand, if the antimony oxide content is over 1 %, the change of the resistance value is small and particularly the antimony oxide content of over 2 % reduces the change of the resistance value to almost naught with resultant superior stability. However, if the antimony oxide content exceeds 10 %, the resistance material will be increasingly melted into the glass and thus bubbles tend to remain in the glass, making it foamy and thus unsuitable to any practical use.

FIG. 2 shows the specific resistance of the binary resistance material in which tin oxide was caused to react with antimony oxide. In FIG. 2, the ordinate represents the specific resistance (k $\Omega$ -cm) and the abscissa represents the amount of the added antimony oxide (%). The ordinate is in the logarithmic scale and the abscissa is in the uniform scale.

As will be seen from FIG. 2, the specific resistance of the resistor comprising the binary system resistance material consisting of tin oxide and antimony oxide is in the very low range of less than 0.00007 k $\Omega$ -cm when the amount of the added antimony oxide is less than 10 %.

However, if tantalum oxide is added as a third constituent to the above-described binary system resistance material, the specific resistance of the resultant material may be increased by about  $10^3$  –  $10^5$  times. The stability of the ternary system resistance material comprising such tin oxide, antimony oxide and tantalum oxide will be described with reference to FIGS. 3 and 4.

FIG. 3 shows the results of the tests conducted according to the load life testing method for automobile spark plugs with resistor defined in JISD 5102 on the resistor composed of the ternary resistance material containing 90 % tin oxide, 5 % antimony oxide and 5 % tantalum oxide and a borosilicate glass mixed with each other in equal proportions. The specific resistance (k $\Omega$ -cm) of the spark plug resistor was checked after the spark discharging over a predetermined period of time. In FIG. 3, the ordinate represents the specific resistance and the abscissa represents the period of spark discharging. In this case, the ordinate and abscissa are both in the logarithmic scales. As will be seen from FIG. 3, the specific resistance of the resistor shows almost no change with increase in the spark discharging period and proves that this spark plug resistor lends itself to be an excellent resistor.

FIG. 4 shows the results of the heat tests conducted on the resistors comprising the above-described ternary

system resistance material according to the method of test for automobile spark plugs with resistor defined in JIS 5102. In FIG. 4, the ordinate represents the specific resistance (k $\Omega$ -cm) and the abscissa represents the temperature (°C) of the resistor and the symbol R indicates the fact that the resistor is at the normal temperature and the specific resistance value indicates the one obtained when the resistor heated to 300°C was cooled to the normal temperature. In FIG. 4, the ordinate is in the logarithmic scale and the abscissa is in the uniform scale.

As will be seen from FIG. 4, the range of variations of the specific resistance is narrow and it is evident that the above-described ternary system resistor for spark plugs according to the present invention meets the specification of JIS 5102 requiring that the tolerance be in the range  $\pm 30$  % of the rated resistance value. The spark plug resistors used in the tests of FIGS. 3 and 4 were cylindrical resistors of the same dimensions.

#### Experimental EXAMPLE 2

The resistance value and specific resistance value of a spark plug resistor comprising a resistance material containing tantalum oxide as its third constituent will be described with reference to FIG. 5.

In FIG. 5, the ordinate represents the resistance value (k $\Omega$ ) of the resistor and the corresponding specific resistance (k $\Omega$ -cm) and the abscissa represents the amount of tantalum oxide (%) in the resistance material.

In FIG. 5, the lines *a*, *b* and *c* are for the compositions where the proportions of tin oxide and antimony oxide differ from one another. Each of the lines represents the specific resistance and resistance value of a resistor in which the above two constituents in predetermined proportions and tantalum oxide are mixed with each other in varying proportions and then bonded with the low melting glass. The line *a* shows the resistance value (and the specific resistance) of the spark plug resistors obtained by using resistance materials comprising a binary system resistance material containing 99 % tin oxide and 1 % antimony oxide and tantalum oxide as a third constitution which are mixed in varying proportions, and mixing each of these resistance materials and the low melting points glass half and half. The line *b* shows the resistance value (and the specific resistance) of the spark plug resistors obtained by using resistance materials comprising a binary system resistance material containing 95 % tin oxide and 5 % antimony oxide and tantalum oxide which are mixed with each other in varying proportions, and mixing each of these resistance materials and the low melting glass half and half. The line *c* shows the resistance value (and the specific resistance) of the spark plug resistors obtained by using resistance materials comprising a binary system resistance material containing 90 % tin oxide and 10 % antimony oxide and tantalum oxide which are mixed with each other in varying proportions, and mixing each of these resistance materials and the low melting glass half and half. The resistors used are of the rod-shaped type having the dimensions of 2.2 mm length and 3 mm diameter.

As will be seen from FIG. 5, the resistance value of the resistor increases in proportion to an increase in the amount of tantalum oxide contained in the resistance material and this tendency remains the same independent of the proportions of tin oxide and antimony oxide

in the resistance material. Further, the higher the tin oxide content is, the higher the resistance value will be. While the line *a* in FIG. 5 represents the cases where the binary systems containing 99 % tin oxide and 1 % antimony oxide are mixed with tantalum oxide, they show the maximum value of tin oxide in the binary systems as mentioned earlier. In each of these cases, the tantalum oxide content in the resistance material should be in the range 1 % or above in order that the resistance value of the resistor may become higher than 3 kilohms. In the cases of the lines *b* and *c* where the tin oxide content is low, the tantalum oxide content of about 2.5 % and above 4 %, respectively, produce the resistors of over 3 kilohms. On the other hand, the line *c* represents the cases where the amount of tin oxide in the binary systems is at the minimum value of 9 %. In each of these cases, the amount of tantalum oxide in the resistance material should be less than 30 % in order that the resistance value of the resistor becomes lower than 20 kilohms. Further, in the cases of the lines *a* and *b* where the tin oxide content is high, it is necessary that the tantalum oxide content be about 30 % and less than 28 %, respectively. It will be seen that by adjusting the amount of tantalum oxide in the resistance material in the range between 1-30 %, the resistor having a resistance value of 3 to 20 kilohms may be obtained. Further, as will be seen from FIG. 6 that will be explained later, this resistance value may also be varied somewhat by varying the amount of the low melting glass mixed with the resistance material.

### Experimental EXAMPLE 3

The change of the specific resistance of the resistor with the variations in the proportions of the low melting glass and the resistance material in the mixtures will be described with reference to FIG. 6. In FIG. 6, the ordinate represents the specific resistance ( $\text{k}\Omega\text{-cm}$ ) and the abscissa represents the weight percent of the glass in the resistor comprising the resistance material and the glass. The resistance material used contained 90.25 % tin oxide, 4.75 % antimony oxide and 5 % tantalum oxide, and this resistance material was mixed with the borosilicate type glass in varying proportions and the mixtures were heated up to about 850°C to produce the rod-shaped resistors whose specific resistances were measured.

As will be seen from FIG. 6, when the amount of the added low melting glass becomes higher than 60 %, the specific resistance increases considerably, whereas the specific resistance does not show any marked change with the glass content of less than 60 %.

The present invention will be described further with reference to the following example.

### EXAMPLE 1

In this example, 95 % of tin dioxide and 5 % of antimony trioxide were mixed and heated with each other in an alumina crucible at a temperature of 1100°C for 5 hours after which the mixture was cooled to the normal temperature. 85 % of this product and 15 % of tantalum pentoxide were intimately mixed and then reacted with each other at 1100°C for 5 hours. The resultant ternary resistance material in granular form was mixed with 50 % of a powdered low melting glass containing borosilicate as its principal element and the mixture added with about 1 % of an organic paste was milled. A given amount of this product was put, as

shown in FIG. 7, in the space above the center electrode 3 in the bore of the insulator 4 and the central conductor 1 was inserted. After heating at 850°C for 30 minutes, a pressure was applied to the central conductor 1 to hot press and seal the product in place where it was firmly held and cooled to provide the resistor 2.

The resistance value of the resistor 2 produced in this way and located between the central conductor 1 and the center electrode 3 was 10 kilohms at the normal temperature while it was 9 kilohms when heated to 400°C. The gastight tests conducted on this spark plug resistor 2 revealed that it was superior showing no leakage even under the applied pressure of 30  $\text{kg}/\text{cm}^2$ . Tests conducted by installing this spark plug in an actual automobile engine showed that the amount of the noise produced was considerably low as compared with that produced by conventional spark plugs equipped with no resistor.

The above-described resistor comprised 50 % of the resistance material containing 80.8 % tin dioxide, 4.2 % antimony trioxide and 15 % tantalum pentoxide and 50 % of the glass.

It will thus be seen from the foregoing description that a spark plug resistor according to the present invention is produced by sintering a resistance material containing 1-30 % tantalum oxide, 63-98 % tin dioxide and 0.7-9.9 % antimony trioxide with a low melting glass, and thus it is possible to provide a spark plug resistor having a resistance value of 3 to 20 kilohms that is essential for the suppression of noises. Particularly, it will be seen that in the resistance material according to the present invention, the specific resistance of the binary resistance material composed of tin dioxide and antimony oxide is increased from below 10  $\Omega\text{-cm}$  up to 100-10,000  $\Omega\text{-cm}$  by a small addition of tantalum oxide as the third constituent and in this way the resistance value of the spark plug resistor can be increased without resorting to any complicated methods by which the amount of glass is increased to obtain an increased resistance value. There is thus a great advantage of providing a resistor which has a narrow range of variations of its resistance value and which is also stable structurally. There is a further advantage that the specific resistance can be easily controlled by adjusting the amount of the added tantalum oxide.

Further, by virtue of the fact that a resistance material is produced by adding tantalum oxide as the third constituent to tin oxide and antimony oxide, there is a still further advantage in that when resistance material is mixed with a glass and heated to produce a sintered mass, the added tantalum oxides ensure a wider range of the sintering temperatures and hence a great convenience in the manufacture of the resistor.

What we claim is:

1. A resistor having a resistance of 3-20 kilohms for a spark plug comprising:

40 to 90 % by weight of a resistance material, said resistance material being composed of tantalum oxide between 1-30 weight percent, tin oxide between 63-98 weight percent and antimony oxide between 0.7-9.9 weight percent, and a glass in an amount of 60 to 10 % by weight for fixing said resistance material.

2. A resistor according to claim 1 wherein the glass is a borosilicate glass.

3. A resistor according to claim 1, wherein the glass is between 20 and 60% by weight of the total of glass and resistance material.

4. A resistor according to claim 1 wherein the antimony oxide is 1 to 10% by weight of the total of tin

5

oxide and antimony oxide.

5. A resistor according to claim 1 wherein the resistance material is 90% by weight tin oxide, 5% by weight antimony oxide and 5% by weight tantalum oxide.

\* \* \* \* \*

10

15

20

25

30

35

40

45

50

55

60

65